

## UNITED STATES PATENT OFFICE

2,103,993

## TREATING CASEIN PLASTICS

Will E. Vawter, Bainbridge, N. Y., assignor to  
American Plastics Corporation, New York,  
N. Y., a corporation of New York

No Drawing. Application October 6, 1936,  
Serial No. 104,299

5 Claims. (Cl. 18—47.5)

This invention has for its object an improvement in the so-called chemical finishing and polishing of shaped objects made from casein plastics, including buttons, blanks, beads, buckles and various others. The art of making casein plastics is so well known that it is not necessary to review the process in this case. After the shaped casein objects have been made by the usual method including the treatment to toughen or harden the same, by means of formaldehyde and preferably after the objects are actually cut, shaped or molded from the casein plastics, it is necessary to give these objects a suitable polish and finish. This was formerly done in tumbling barrels by means of pumice, waxes and the like, a process well known to the art for many years, not only in the casein plastics art but in the ivory nut button art. Of late years it has been found possible to treat the casein objects in a chemical bath to obtain the desired polish and finish and thus not only improve the final casein objects, but reduce the cost of the polishing process and the time required therefor, to a very large extent. The principle of the chemical polish is well known in the industry and there are a number of these chemical polishing compounds regularly sold on the market. In general the chemical finishing and polishing substances consist of an alkali hypochlorite or a mixture of several alkali hypochlorites, or an alkaline earth hypochlorite, or mixtures of various alkali and alkaline earth hypochlorites and such products will be referred to for the purpose of this case as "chemical polish". I have found that there is a considerable variation in these chemical finishing compounds as to speed of reaction, strength of solution and therefore variations in the finished chemically polished casein objects. The usual procedure heretofore in factory practice for chemically polishing casein objects has been as follows:—

To 150 parts of water by weight, there is added 25 parts by weight of commercial "chemical polish" (i. e. hypochlorite solution containing about 47 to 51 grams of available chlorine per liter). Casein plastic objects are added to this hot solution and are agitated therein by any convenient means for about 4 minutes. They are then well washed, preferably several times (e. g. three times) with hot water, at about 140° F. to 150° F. The objects are then dried by any convenient means, e. g. in the air or in low temperature drying tunnels, preferably while being agitated. After following this process it will be noted that the casein objects which previous to the chemi-

cal polish treatment, possessed a dull, unpolished surface, after the treatment possess a shiny, smooth, gloss-like finish.

I have discovered however, that there are several serious defects resulting from the above method of chemically polishing casein objects. One objection is that after the above described treatment the objects come out of the final wash water in rather a slightly sticky condition so that the objects are apt to stick together. They have rather a soft slimy feel. Furthermore, the most serious disadvantage by using this process resides in the fact that this chemical polish treatment often changes the shade of the casein objects. And not only is this changing of shade a serious drawback but it is still more serious from the fact that different batches of casein objects, buttons for example, which have been treated by this chemical polish, will not all be exactly the same shade, or do not precisely match the color shade desired. I have noticed in making five different batches of chemically polished brown buttons, the buttons having been dyed with the same brown aniline dye during the process of making the casein buttons, and applied in the same way, under like conditions, that the shade in each of the five batches was different. I believe that the reason for this is the fact that very slight changes in temperature of the solution of the chemical polish, or a slight difference in the length of time in which the buttons were immersed in the chemical polish solution, or a slight difference in the final washing of the different finished batches, may be the cause of this variation in shade. It can be well understood that such variations in shade of different batches in the same lot of buttons of casein objects, is a very serious matter and in many cases would compel one to place these various batches of off-shade finished buttons into another shade class, or to dispose of them as seconds or to re-dye these buttons, because of this non-uniformity.

My invention consists in a subsequent treatment of the chemically polished casein objects (polished in hypochlorite solution) in such a manner that even though the shades up to the point of the casein objects having been chemically treated and washed, are varied, yet by my process I can bring them back to the original shade of color so that they will then be all of the original or substantially original shade that they had prior to the chemical polishing treatment. To accomplish this improvement in the art of chemically polishing casein objects I give

herewith by way of illustration, my preferred method which is substantially as follows:

The buttons or casein objects are given the chemical polish (hypochlorite treatment) and 5 washing substantially as described above or by any usual known factory method (using hypochlorite or equivalent), up to the point of having finished the washing operations. After the washing I immerse the chemically polished buttons or casein objects in a weak, hot acid solution and allow these buttons or casein objects to remain in this solution for a few minutes, preferably with agitation. They are then removed and washed preferably in two wash waters, the water 10 being at a temperature of about 140° F., removed from the wash water, drained and dried by the usual method. By this process I find that these buttons or casein objects will regain the exact shade or substantially the exact shade which they 15 possessed prior to having given them the chemical polish treatment and furthermore when the buttons or casein objects are treated by my method they have a brighter, clearer appearance than those not so treated, but treated by the 20 usual chemical polishing treatment.

I have carried on a great many experiments with various types and kinds of acids and at various strengths and I have also made many tests with other organic and inorganic chemical 25 compounds including many acid salts and/or alkali-neutralizing salts, and I find that what seems to be the most desirable and cheapest and yet highly effective way to accomplish these results is with a weak solution of an inorganic acid, 30 although I am able to obtain quite satisfactory results with various organic acids, but the time required to accomplish the results seems to be longer than with the mineral acids. I have also found that a number of the acid salts give quite 35 satisfactory results.

In practicing this invention I do not wish to limit myself to any particular strength of acid or acid salts, although I have found very satisfactory results are obtained with very weak solutions. In order that one skilled in the art may 40 practice my invention I give herewith one typical commercial example as to the method that can be followed:—

#### Example 1

50 Into a proper tank, tub or mixer, I add 150 gallons of water and 2 gallons of ordinary commercial sulfuric acid of about 93% strength. This acid solution is heated to 150° F. and I then put into the mixture 100 lbs. of casein buttons or other moulded or shaped casein objects (which have been polished by treatment in the above described hypochlorite treatment). The temperature is kept at approximately 140° F. for say, 10 55 minutes, and the immersed objects are gently stirred or tumbled in this acid solution during the treatment. The buttons or casein objects are then removed and are thoroughly washed, preferably giving two washings with water at about 140° F., while agitating. The objects are then drained and dried and it will be noted that the buttons or casein objects thus treated have returned to the exact shade or substantially the 60 exact shade of the material prior to the chemical polish (hypochlorite) treatment. It is also found to be possible to obtain about the same results without heating the acid solution but it requires a much longer time and it is to be understood 65 that other proportions or concentrations of the 70

acid may be used without departing from the object of this invention.

Other examples which have given satisfactory results are as follows:—

#### Example 2

150 gals. of water, 2 gallons concentrated hydrochloric acid of 37%, of the ordinary commercial grade. Proceed as in Example 1. .

#### Example 3

150 gallons of water, 4 gallons nitric acid of 70%, and the ordinary commercial grade. Proceed as in Example 1.

#### Example 4

150 gallons water, 2 gallons 35% formic acid. Proceed as in Example 1. The final results are quite satisfactory but the time required for the casein objects to remain in the acid bath is somewhat longer. A treatment for 15-20 minutes is recommended, when using formic acid.

#### Example 5

150 gallons of water, 2 gallons glacial acetic acid. Proceed as in Example 1. The results are entirely satisfactory, but the length of time required in the acid bath is somewhat longer than in Example 1, 12 to 15 minutes being satisfactory.

#### Example 6

150 gallons of water, 2 gallons lactic acid 85% purity. The results are satisfactory but the period required is somewhat longer than in Example 1. About the same results are secured as in Example 5.

#### Example 7

150 gallons of water, 2 gallons phosphoric acid approximately 85% purity. These results are entirely satisfactory; the length of time in the acid bath being somewhat shorter than Examples 4, 5 and 6 and a little longer than Example 1, say 12 minutes.

#### Example 8

150 gallons water, 2 gallons hydrofluoric acid 30% strength. Results satisfactory but the time in the acid bath is somewhat longer than in Example 1, say 15 minutes.

#### Example 9

150 gallons of water, 2 gallons hydrofluosilicic acid 30% strength. The results are satisfactory but the time in the acid bath was approximately twice as long as in Example 1.

In place of the acids mentioned in the examples, other acids, acid salts or substances capable of neutralizing alkalies, can be used. For instance I may mention oxalic acid 1.3 to 2%, propionic acid 1.5 to 2.5%, potassium bisulphite 60 or sodium bisulphite 1.5 to 3%, tartaric acid 1.5 to 2.5% (applied for say 5 to 15 minutes) or other substances such as trichloracetic acid, barbituric acid, succinic acid, disodium phosphate, monocalcium phosphate, potassium bitartrate, glycerol phosphoric acid, malic acid, ammonium persulphate, aluminium sulphate or chloride, can also be employed, but in somewhat greater concentration than given above, and/or continuing for a longer time. Ferric sulphate was found to restore the 70 color rapidly, but gave a somewhat dull finish.

The process is applicable not only to casein products containing anilin dyes, but also to a wide variety of other dyes. It will be understood however that when using casein plastics containing 75

5 a particular dye, it is advisable to ascertain the concentration of the acid or acid salt that is best suited for that particular dye. The concentrations given in the examples are based on soluble anilin dyes, and particularly acid dyes (mixed with the casein before extrusion, if desired), or mixtures of these and other dyes. It is to be understood that concentrations, times, temperatures of the acid treating bath are not limited to 10 the details given in the examples. The concentrations here given are such as will give a good color restoration within a few minutes, and without any apparent injury to the articles treated. The temperatures of 140 to 150° F. are preferred, 15 but the solutions will be operative even at room temperature, although much slower. In many instances, substantial restoration of the color could be secured in half the time stated above.

It should be noted that the change of color 20 (during the hypochlorite treatment and acid treatment) referred to in this specification applies not only to casein objects which have been made with various water soluble dyes, but it also applies to casein objects which have been colored 25 with pigments of various types, as well as to casein objects of a white type containing white pigments and to casein objects which contain no dye or no pigments, known as "blond" type. Where casein buttons or casein objects are made 30 white by mixing into the casein at the time the casein plastic is made, various white pigments and then preparing the casein objects from such finished casein plastics and polishing by means of a chemical polish, I find that these white casein 35 objects assume a yellowish cast and where the casein plastics have been made without the addition of any pigment or dye and thus produces what is known as a "blond" casein object and such casein plastic is made into objects and chemically 40 polished, I find that such objects take on a yellowish cast but when any subsequent acid treatment is given to the white or the "blond" casein objects, they resume their natural shade.

45 My invention involves a process of improving the chemical polish or chemical finish of casein plastic objects substantially as described in this specification, by treating said objects after chemically polishing, with a water soluble acid reacting substance capable of restoring the fading of color or change of color caused by the chemical polishing process.

50 For testing this process, a variety of differently colored batches of discs, stamped out of a casein plastic sheet have been treated by this process. 55 In a particular series of tests, a casein plastic

sheet was used, in which the moistened rennet casein was well mixed with a dye mixture consisting of Leather brown EG, Nigrocene crystals and Cloth red B extra. The mixture was then extruded, pressed into a thin sheet and dried, and the discs stamped out, formalized and then treated with a sodium hypochlorite solution containing about 7% of available chlorine, for giving the "chemical polish". The action of this latter solution caused a decided reddening of the discs, 10 which before that treatment were of a deep chocolate brown color. The treatment as described restored the original color.

15 It may be stated that acid dyes of all colors are generally suitable for giving the desired color to casein plastics. Certain basic dyes have also been used. For giving the desired color, it is common to use a mixture of several different dyes.

I claim:—

1. A process of treating shaped casein plastics 20 having a predetermined color, which comprises first polishing said articles by subjecting same to the action of a hypochlorite solution to polish the same whereby the color is injured and the surface rendered slimy, and thereafter to the action of a 25 solution having a weak acidic reaction, to restore the color.

2. A process of treating shaped casein plastics having a predetermined color, which comprises first subjecting same to the action of a hypo- 30 chlorite solution to polish the same, and thereafter subjecting the same to the action of a dilute mineral acid solution.

3. A process of treating shaped casein plastics having a predetermined color, which comprises 35 first subjecting same to the action of a hypochlorite solution to polish the same, and thereafter subjecting said articles to the action of a dilute organic acid solution.

4. A process of treating shaped casein plastics 40 having a predetermined color, which comprises first subjecting same to the action of a hypochlorite solution to polish the same, whereby the surface becomes discolored, and thereafter subjecting said plastics to the action of a solution of 45 an acid salt, whereby the color is restored.

5. A process of treating shaped casein plastics having a predetermined color, which comprises first subjecting same to the action of a hypochlorite solution to polish the same, whereby the 50 surface becomes discolored, and thereafter subjecting said plastics to the action of dilute sulphuric acid, whereby the color is restored.

WILL E. VAWTER. 55